

## UNITED STATES PATENT OFFICE

2,320,984

## LUBRICATING COMPOSITION

Carl F. Prutton, East Cleveland, Ohio, assignor, by  
mesne assignments, to The Lubri-Zol Develop-  
ment Corporation, Cleveland, Ohio, a corpora-  
tion of Delaware

No Drawing. Application December 4, 1934,  
Serial No. 755,987

15 Claims.

(Cl. 252—53)

This invention relates as indicated to lubricating compositions and in one form comprises the combination of a suitable oil base and certain addition agents for the purpose of improving the lubricating properties of such oil base and more particularly to impart extreme pressure characteristics to such composition.

As disclosed in my co-pending application Serial No. 638,599 filed October 19, 1932, certain desirable improvements in the lubricating properties of a lubricating oil may be secured by the combination therewith of certain halogenated additions, particularly halogenated or more specifically chlorinated organic compounds.

The present invention relates to the combined use in a lubricating composition of organic oxygen bearing compounds and organic halogen bearing compounds.

I have discovered that certain oxygen-bearing organic compounds in combination with a mineral oil base which also has added thereto certain organic halogen bearing compounds produce a lubricating composition equal to and, in certain respects, superior to the result secured by the use of a pure hydrocarbon oil as a lubricant or a composition including in combination a pure hydrocarbon oil and certain addition agents such as organic halogen bearing compounds. The lubricating composition according to my present invention is particularly applicable for use as an extreme pressure lubricant.

For a definition of extreme pressure lubrication and the distinction thereof over low pressure or thick film lubrication reference may be had to the specification of my above mentioned co-pending application.

It is among the objects of my invention, therefore, to provide a lubricating composition which shall be superior to any which has heretofore been available. Other objects of my invention will appear as the description proceeds.

To the accomplishment of the foregoing and related ends, said invention, then, consists of the features hereinafter fully described, and particularly pointed out in the claims, the following description setting forth in detail certain embodiments of the invention, these being illustrative, however, of but a few of the various ways in which the principle of the invention may be employed.

Particularly stated, this invention comprises

the combined use as a lubricating composition of organic oxygen bearing compounds and organic halogen bearing compounds and the combined use of both of such materials as addition agents to lubricating compositions which also contain a suitable lubricating oil such as mineral oil.

I have found that while the addition of a halogen in the form of an organic compound generally improves the lubricating properties of a mineral oil, nevertheless, when such halogen is present in the form of certain of the available halogenated organic compounds it is so strongly combined that when used alone as an addition agent to a mineral oil, the extreme pressure characteristics of the composition are not as improved as may be desired for certain uses. The additional presence of oxygen in such oxygen compositions, however, renders such halogen more active so that the extreme pressure characteristics of the composition are considerably better than that secured by the use of a halogen alone.

The oxygen referred to above may be conveniently present in the composition in the form of oxygen containing or bearing organic compounds. Both the halogen bearing organic compounds and the oxygen bearing organic compounds for purposes of convenience, may be classified as follows:

- 30 I. Aliphatic, or carbon chain type
  - A. Derivatives of hydrocarbons of the paraffin series,
  - B. Derivatives of hydrocarbons of the olefine series
  - and
  - C. Derivatives of hydrocarbons of the acetylene series.
- II. Organic ring type
  - 35 A. "Carbon ring" type compounds
    - (a) Of the aromatic, or allied type, including derivatives of benzene, naphthalene, an-  
thracene, etc., also compounds of the  
bridged ring type, such as the terpenes,  
and related compounds.
    - (b) Of the class including the cycloparaffins,  
cyclo-olefines, etc. Examples of this class  
are derivatives of the following:
      - (1) Hydrogenation products of ben-  
zene (e. g. cyclohexane, cyclo-  
hexene, cyclohexadiene).
      - (2) Hydrogenation products of naph-  
thalene (e. g. decahydronaphtha-  
lene, etc.).
      - (3) Naphthenes, naphthenic acid,  
etc.
    - (c) Of mixed type such as derivatives of in-  
dene, hydrindene, hydranthracene, etc.
  - B. "Heterogeneous ring" type compounds
    - (a) Of the aromatic or allied type including de-  
rivatives of pyridine, quinoline, etc.
    - (b) Other types such as a furan and its deriva-  
tives and derivatives of thiophene, pyr-  
role, etc.

The oxygen bearing derivatives of the foregoing compounds may also be classified according to the nature of the attachment of the oxygen to the molecule viz.:

I'. Directly attached to one or more carbon atoms, as in the case of:

- (1') Ethers and analogous compounds
- (2') Compounds containing the  $=C-OH$  radical, such as alcohols and other derivatives of carbinoi (including phenols, cresols, naphthols etc.)
- (3') Compounds containing the carbonyl ( $\equiv C=O$ ) radical, such as aldehydes, ketones, organic acids, esters and salts of organic acids, thio-acids and esters of thio-acids.
- (4') Compounds in which oxygen forms a part of the ring structure, e. g. furan and its derivatives, anthraquinone, etc.

II'. Indirectly attached through the means of some other atom, i. e., in the form of an inorganic radical, e. g.:

|               |                |    |
|---------------|----------------|----|
| Amide         | Oxime          | 5  |
| Arsenate      | Perchlorate    |    |
| Arsenite      | Phosphate      |    |
| Chlorate      | Phosphite      | 10 |
| Chlorite      | Sulphate       |    |
| Cyanate       | Sulphite       |    |
| Hydroxylamine | Sulphinic acid |    |
| Hypochlorite  | Sulphone       |    |
| Nitrate       | Sulphonic acid |    |
| Nitrite       | Sulphoxide     | 15 |
| Nitro         | Thio-phosphate |    |
| Nitroso       | Thio-sulphate  | 25 |

Of the above enumerated compounds the carboxylic acids and the esters and salts of such acids are preferred, e. g., fatty oils, vegetable oils, oleic acid, stearic acid, amyl acetate, butyl stearate, dibutyl phthalate, methyl salicylate, naphthenic acid, butyl naphthenate; sodium, calcium and aluminum stearates and oleates; sodium, calcium and lead naphthenates, aniline stearate, aniline oleate, stearanilid, quinoline oleate, quinoline stearate.

The halogenated organic compounds employed in accordance with this invention are preferably halogenated carbon ring compounds which are preferably of the chlorinated species and particularly the following compounds have been found to produce very satisfactory results, viz.:

Halogen bearing derivatives of:

I. Benzene, such as:

- (1) Halogenated benzene, e. g.
  - (a) Monochlorbenzene
  - (b) The dichlorbenzenes, notably the ortho compound
  - (c) The trichlorbenzenes, notably the 1, 2, 4 compound

(2) Halogenated derivatives of benzene such as

- (a) Halogenated homologs of benzene, e. g.
  - Chlorinated toluene
  - Chlorinated xylene
  - Chlorinated cymene

- (b) Halogenated amino derivatives of benzene, e. g.
  - Chlorinated aniline
  - Chlorinated toluidines
  - Chlorinated xylydines

- (c) Halogenated hydrobenzenes, e. g.
  - Dichlorhexahydrobenzene (dichlor cyclohexane)

II. Diphenyl, diphenyl benzenes, such as:

- (1) Chlorinated diphenyl
- (2) Halogenated derivatives of diphenyl, such as,

- (a) Halogenated homologs of diphenyl, e. g.
  - Chlorinated phenyl-toluenes

- (b) Halogenated amino derivatives of diphenyl, e. g.
  - Chlorinated phenyl-anilines
  - Chlorinated phenyl-toluidines

- (c) Halogenated hydrodiphenyls, e. g.
  - Chlorinated phenyl hexahydrobenzene
  - Chlorinated dodecahydrodiphenyl

III. Naphthalene, such as:

- (1) Chlorinated naphthalene
- (2) Halogenated derivatives of naphthalene such as:
  - (a) Halogenated homologs of naphthalenes, e. g.
    - Chlorinated methyl naphthalene notably the alapha compound,
    - Chlorinated propyl, and isopropyl substitution products of naphthalene
  - (b) Halogenated amino derivatives of naphthalene, e. g.
    - Chlorinated naphthylamines
  - (c) Halogenated hydronaphthalenes, e. g.
    - Chlorinated decahydro-naphthalene

IV. Phenanthrene and anthracene, such as:

- (1) Chlorinated phenanthrene, chlorinated anthracene
- (2) Halogenated derivatives of phenanthrene and anthracene, such as—
  - (a) Halogenated homologs, e. g.
    - Chlorinated 1 - methyl phenanthrene
    - Chlorinated 3 - methyl phenanthrene
    - Chlorinated 9,10 - methyl phenanthrene
    - Chlorinated propyl and isopropyl derivatives of phenanthrene such as retene
    - Chlorinated  $\alpha$ -methyl anthracene
    - Chlorinated  $\beta$ -methyl anthracene
    - Chlorinated dimethyl anthracenes
    - Chlorinated propyl and isopropyl substitution products of anthracene
  - (b) Halogenated amino derivatives, e. g.
    - Chlorinated phenanthryl-amines
    - Chlorinated anthramines
  - (c) Halogenated hydrophenanthrenes and halogenated hydronaphthalenes

V. Chrysene, and picene.

It will be noted that the above enumerated examples of carbon ring compounds which are preferably employed are compounds of the aryl type, i. e., compounds containing benzenoid ring structures and are also of the type in which the halogen is directly attached to an atom which is 75 a part of such ring structure.

Compounds of types related to certain of the above are also particularly useful such as halogen bearing derivatives of pyridine quinoline, pyrrole, thiophene and furan.

As a matter of convenience, the halogenated diphenyls and substituted diphenyls, as well as halogenated substituted benzenes where two or more phenyl groups are directly linked may be inclusively referred to as halogenated polyphenyls.

The base of the lubricating composition may be, as previously indicated, any oily material, preferably mineral oil; however, other material such as fixed oils, and special oils such as sulphur-treated oils, may be advantageously employed for particular purposes. The optimum amount of the addition agents to be employed in conjunction with the oil base as above defined, will depend upon the particular character of such compounds, i. e., their physical characteristics and especially their effect upon the viscosity of the oil to which the same are added. The particular use for which the lubricant is intended is also a governing factor in determining the amount of the compound or compounds to be added.

My invention, as above explained, contemplates the addition to a suitable oil base of minor amounts of addition agents in such proportions as not to materially reduce the viscosity of the oil. Since the loss of such addition agents by volatilization will in general be less for higher boiling material, the boiling point of the addition agents should be at least 125° C. and preferably above 140° C.

It is to be understood that the so-called "addition agents" referred to herein shall be substantially oil-soluble or of such nature that they may be included in the composition in the form of a stable colloidal suspension. It should also be noted that certain of the addition agents contemplated by this invention, while soluble in oil do not dissolve readily therein. When such compounds are used they may be first dissolved in materials such as, benzene, the chlorbenzenes, the higher alcohols such as amyl alcohol, acetone, petroleum naphtha, carbon tetrachloride, tetrachlorethylene, aniline, tricresyl phosphate, etc., and the resulting solution then added to the lubricating composition.

In the case of organic oxygen compounds which are very strongly adsorbed by metal surfaces (e. g., fatty acids and derivatives of them) if too much is added, the halogen compound may be prevented from functioning to increase the film strength, probably by being displaced from such surfaces. It is, therefore, advisable to determine the amount of the oxygen compound used which will have the optimum effect.

In general, the lubricating composition, in accordance with my invention, may comprise the so-called addition agents in their pure state or with a minor amount of mineral oil added thereto; however, for most uses, a composition comprising a major proportion of a suitable oil base and a minor proportion of the addition agents will be found most satisfactory.

An example of a composition comprising such addition agents in their pure state without the addition of a mineral oil would be a mixture of chlorinated diphenyl and an ester of stearic acid, for example, butyl stearate. In this case on account of the high viscosity of the organic halogen compound, no mineral oil is required for "thick-film" lubrication, and the improved re-

sults due to the presence of oxygen may be obtained by the sole addition of such organic oxygen compounds, usually in minor amounts.

As above pointed out, the halogenated organic ring compounds are preferred over the halogenated open chain compounds as the source for the halogen or more specifically, the chlorine. The reason for such preference is that chlorine is sufficiently stable in the ring compounds so that in the presence of water there will be no appreciable amount of hydrolysis which would result in corrosion of the metal parts with which the composition comes in contact. In the form of the ring compounds, the chlorine is sufficiently closely combined so that it will become available to chemically react with the bearing surfaces to produce the desired results only under the conditions imposed by the relative movement between such surfaces. In certain of the ring compounds, however, the chlorine is so closely attached that it is not made sufficiently available for the desired results, even under the conditions imposed by the relative movement between the bearings. The additional presence of oxygen, however, cures this difficulty and it is this reason, among others, which may explain the unusual and unexpected results secured by the combined use in the composition of the oxygen and chlorine.

This invention also contemplates the use in lubricating compositions of halogenated carbon chain compounds and a separate organic oxygen bearing compound for the purpose of increasing the film strength. Such compositions are especially useful where unusually extreme conditions of pressure exist, the activity of the halogen being further increased, as in the case of the ring compounds, by the addition of organic oxygen compounds thus increasing the range of usefulness of such compositions.

Of the chain compounds which may be employed, such as hexachlorethane, acetylene tetrachloride, butylene dichloride (1-2 di-chlorbutane), monochlorhexane, 1-2 dichlor hexane, amylene dichloride, etc. or any other halogen substitution or addition products of the paraffins, olefines or acetylenes or derivatives of them, the less volatile and more stable are preferred for the reasons above set forth. Certain halogenated commercial products which are mixtures of such compounds are also adapted for this use, such as: chlorinated wax, chlorinated kerosene, chlorinated motor oil, etc.

For the purpose of lubricating and reducing the friction between the relatively moving parts of an internal combustion engine, such as crank case bearings, piston and cylinder surfaces, as well as piston rings and valves, the composition will preferably comprise a major proportion of an oil base such as mineral oil and concentrations of from  $\frac{1}{10}$  of 1% to 2% of the addition agents. If the valve structure of such engine is to be lubricated separately from the remainder of the engine or by means connecting in an auxiliary fashion, the lubricating composition will preferably contain a larger amount of such addition agents, i. e., from about 2 to 10%.

The lubricating compositions referred to herein have a particular advantage in the tendency of the compounded lubricant employed to keep down carbon formation and hence, such compositions are particularly applicable for the lubrication of the upper parts, i. e., pistons, valves, piston rings, etc. of an internal combustion engine by dissolving the specified composition in

the motor fuel, so that such fuel when introduced into the combustion chamber is volatilized and the lubricating composition will be distributed over the walls of such chamber as well as the valves and their associated parts.

The composition comprising my invention has certain advantages when used as a lubricant of which the following may be mentioned:

*First.*—By the use of this composition, it is possible to extend the pressure range between the bearing surfaces because of the reduced tendency for bearing surfaces so lubricated to become scored or to seize at higher pressures than are allowable with ordinary lubricants.

*Second.*—The friction between the bearing surfaces is reduced, especially in the higher pressure range, below that obtained with ordinary lubricants.

This application is a continuation-in-part of co-pending applications, viz: Serial Number 649,734, filed December 31, 1932 and Serial Number 737,070, filed July 26, 1934.

Other modes of applying the principle of my invention may be employed instead of the one explained, change being made as regards the materials employed in carrying out the process, provided the ingredient or ingredients stated in any of the following claims or the equivalent of such stated ingredient or ingredients be employed.

I therefore particularly point out and distinctly claim as my invention:

1. A lubricant compound of high film strength and lower coefficient of friction, over a significant range of working conditions, than any one of its constituents or any two of its constituents combined, comprising a major proportion of mineral lubricating oil, a minor proportion of a substantially neutral, body of oil-film strengthening, oil-soluble, aromatic hydrocarbon having chlorine in chemical combination therewith of the type illustrated by chlor-naphthalene and chlor-diphenyl, said body substantially non-volatile at ordinary temperatures, and a minor proportion of another body of friction-reducing, oil-soluble organic compound having oxygen in saponifiable chemical combination therewith, the total proportion of said bodies being within the limit of their combined solubility in said lubricating oil.

2. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble organic oxygen compound, the total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen and oxygen compounds respectively have been omitted.

3. A lubricating composition containing as a principal lubricating constituent a major amount of mineral lubricating oil with the properties of such composition affecting its use as a lubricant improved by incorporating therein an effective minor amount of both an oil-soluble halogenated

carbon ring compound and an oil-soluble organic oxygen compound, the total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen and oxygen compounds respectively have been omitted.

4. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble organic oxygen compound, the total proportion of said compounds being within their combined solubility in said mineral lubricating oil and said compounds being of the type having a vapor pressure less than atmospheric at a temperature of 140° C., and said lubricant characterized by a higher film strength or lower coefficient of friction respectively, over a significant range of working conditions, than similar lubricant compounds from which said halogen and oxygen compounds respectively have been omitted.

5. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble ether, the total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen and oxygen compounds respectively have been omitted.

6. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble organic carbonyl compound, the total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen compound and said oxygen compound respectively have been omitted.

7. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble ester, the

total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen and oxygen compounds respectively have been omitted.

8. A lubricating composition containing as a principal lubricating constituent a major amount of mineral lubricating oil with the properties of such composition affecting its use as a lubricant improved by incorporating therein an effective minor amount of both an oil-soluble halogenated organic compound and an oil-soluble ketone, the total proportion of said compounds being within their combined solubility in said mineral lubricating oil and said compounds being of the type which will not substantially evaporate from such lubricating composition at ordinary temperatures, and said lubricant characterized by a higher film strength or lower coefficient of friction respectively, over a significant range of working conditions, than similar lubricant compounds from which said halogen and oxygen compounds respectively have been omitted.

9. A lubricating composition consisting entirely of the combination of an oil-soluble halogenated organic compound and an oil-soluble organic oxygen compound, the proportion of said compounds being within their mutual solubility and said compounds being of the type having a vapor pressure 35

less than atmospheric of a temperature of 140° C., and said lubricant characterized by a higher film strength or lower coefficient of friction respectively, over a significant range of working conditions, than said halogen and oxygen compounds, respectively, when used alone.

10. A lubricant composition comprising a solution of an oil-soluble halogenated organic compound and an oil-soluble organic oxygen compound, said compounds being present within the limit of their mutual solubility and of the type having a vapor pressure less than atmospheric at a temperature of 140° C., said composition being effective to provide a lubricant having a higher film strength or lower coefficient of friction respectively over a significant range of working conditions, than similar lubricants from which said halogen compound and said oxygen compound respectively have been omitted.

20 11. A composition in accordance with claim 2 in which the halogenated organic compound is an aromatic compound.

12. A composition in accordance with claim 2 in which the halogenated organic compound is orthodichlor benzene.

25 13. A composition in accordance with claim 2 in which the halogenated organic compound is a cycloaliphatic compound.

14. A composition in accordance with claim 2 30 in which the halogenated organic compound is a derivative of cyclohexane.

15. A composition in accordance with claim 2 in which the halogenated organic compound is chlorinated decahydronaphthalene.

CARL F. PRUTTON.